

## UNITED STATES PATENT OFFICE.

ROBERT JOHN, OF NEW YORK, N. Y., ASSIGNOR TO DAYLIGHT FILM CORPORATION, A CORPORATION OF NEW YORK.

PROCESS OF MAKING A CONTACT TRANSFER PRINTING SURFACE WITH A COLORED EMULSION.

No Drawing. Application filed October 23, 1919. Serial No. 332,806.

To all whom it may concern:

Be it known that I, ROBERT JOHN, a citizen of the United States, residing at New York, in the county of New York and State of New York, have invented certain new and useful Processes of Making a Contact Transfer Printing Surface with a Colored Emulsion, of which the following is a specification.

10 My invention relates to a process of making a contact transfer printing surface with a colored emulsion and has for its object to produce a printing surface which is mounted on a suitable carrier and which represents 15 photographic lights and shades in such a manner that copies may be made therefrom by a dye or ink transfer contact process. An illustrative dye contact transfer process is disclosed in patent to Shepherd and Bartlett, No. 728,310, granted May 19, 1903, for 20 photographic printing, and an illustrative ink contact transfer process is disclosed in Cassell's Cyclopædia of Photography, Cassell & Co., New York, 1912, at page 124 25 under the title "Collotype", it being understood, however, that the processes thus illustrated do not disclose a printing plate having the novel and beneficial characteristics of the printing plate obtained by the 30 process disclosed and claimed herein. More specifically, my invention relates to the formation of a printing surface obtained by exposing to the action of light modified by the lights and shades which it is desired 35 to reproduce, a sensitized emulsion mounted on a transparent carrier through which it preferably is exposed, which then is treated to form a hardened printing surface consisting of granules or great numbers 40 of photographically formed, extremely minute, individual protuberances which are distributed and grouped irregularly so as to represent photographic lights and shades. The exposure light may be of any kind, 45 such for example, as a reflected light as in a camera, or a transmitted light as in printing from a negative.

In the embodiment of my invention chosen for purposes of illustration, the printing surface referred to may be obtained by the process described in my Patent No. 1,374,853, granted April 12, 1921, 50 for process of photographic reproduction.

In accordance with that process, the exposed emulsion may be treated by a developing solution containing a hardening or tanning agent which renders insoluble or unremovable the emulsion adjacent its light affected, light sensitive content, the effect of which agent is controlled or limited 55 selectively by the presence of varying quantities of a neutralizing agent, after which the soluble or removable portions of emulsion are removed in any desired manner, as, for example, by melting with warm 60 water.

A sample formula for a developing solution containing a hardening or tanning agent the effect of which is controlled and limited selectively by the presence of varying 70 quantities of a neutralizing agent is as follows:

|                   |                 |
|-------------------|-----------------|
| Water             | 8.5 ounces      |
| Pyrogallic acid   | 11 grains 75    |
| Metol             | 9 grains        |
| Potassium bromide | 4 grains        |
| Sodium carbonate  | 200 grains      |
| Sodium sulphite   | 40 to 60 grains |

In the above sample formula the hardening or tanning agent is pyrogallic acid, and the controlling and limiting agent is sodium sulphite which may be varied in amount selectively within limits to obtain the desired result. It is well known that pyrogallic acid 80 also is a developing agent and that sodium sulphite is a preservative adapted to prevent oxidation of the pyrogallic acid in solution. Other hardening and tanning agents and other neutralizing agents may 85 be used, the above formula representing one developing solution by which the process may be carried out. Potassium bromide, for example, also has a certain controlling and limiting effect. The main difference 90 between the above sample formula and standard developing formulas is in the amount of sodium sulphite used. In standard formulas the amount of sodium sulphite used is so 95 greatly in excess of the amount used in the 100 above sample formula that the tanning or hardening effect of the pyrogallic acid is entirely neutralized or overcome. In the sample formula, the sodium sulphite merely controls and limits the hardening effect of the 105 pyrogallol. It is of course understood by

those skilled in the art that when a thick layer of emulsion is treated, or when the exposure is through the transparent carrier, it is advisable, in order to accelerate the action of the pyrogallic acid, to use larger quantities of an accelerator such, for example, as sodium carbonate or its equivalents than when the emulsion layer is thin or exposed on its face. When larger quantities of sodium carbonate thus are used, it is necessary to increase the amount of sodium sulphite. The above sample formula is for treatment of an emulsion exposed through its transparent carrier and therefore contains a comparatively large amount of sodium carbonate with an increased amount of sodium sulphite. In order to obtain the desired printing surface, however, the amount of sodium sulphite in the process disclosed herein is much less than would be used in a developing solution for the usual development of the particular emulsion layer to be treated. Although it is preferable for reasons of convenience to embody the selectively controlled hardening agent in the developer solution, it may be used separately if desired, by such modification of the developer solution as will prevent such a hardening of the emulsion as will prevent the selective hardening desired.

It is believed that the hardening or tanning effect of the pyrogallic acid exerts its action first adjacent the so-called latent image, or in other words, on the portions of emulsion adjacent the particles of silver salts affected by the exposure light and converted by the developer into metallic silver. Thus in a silver bromide film, the throwing off of the bromide from a light affected silver bromide particle in the developing process, probably acts or reacts with the pyrogallic acid to harden or tan or render insoluble or unremovable the adjacent emulsion. Thus in the embodiment chosen for purposes of illustration, the reaction products from the chemical effects of the developer solution, are believed to act or react with the selectively controlled hardening agent. However this may be, it is necessary for purposes of my invention as disclosed in said Patent No. 1,374,853, dated April 12, 1921, only either to harden particles of emulsion adjacent light affected particles of the light sensitive content in any desired manner, or in reverse manner to leave unhardened the particles of emulsion adjacent light affected particles of the light sensitive content and harden the remaining emulsion, the essential result being a hardened emulsion surface corresponding to the lights and shades to be reproduced which will acquire and give up any desired color in a comparatively short time. By controlling the hardening or tanning effect of the pyro-

gallic acid as above set forth, only the particles of emulsion adjacent the said light affected particles of silver salts are hardened, the relative proportions of the hardening agent (whether or not accelerated by an accelerating agent) and of the neutralizing agent being such as to control selectively the effective area of influence of the hardening agent. The unhardened portions, as stated above, then may be removed in any desired manner as by placing the emulsion in warm water which causes the unhardened or soluble portions to soften and melt away from the hardened or insoluble portions so that the hardened emulsion alone will remain in the form of extremely minute, individual protuberances which are distributed and grouped irregularly so as to represent the photographic lights and shades which it is desired to reproduce. 85

It is considered desirable in producing a printing surface to expose the sensitized emulsion through its transparent carrier rather than on its outside surface in order that the printing surface may be as close as possible to the carrier. If the emulsion is exposed on its outside surface, it is necessary to strip the emulsion from its carrier in order to remove the unhardened portions which will lie adjacent the carrier. Stripping the emulsion is a delicate operation which can be performed only by those skilled in the art and is likely to injure the image.

When an emulsion is exposed through its transparent carrier, however, certain difficulties are encountered in the formation of the printing surface, which preferably should be very thin and lie adjacent the transparent carrier. As an ordinary commercial sensitized emulsion usually is in excess of one-thousandth of an inch in thickness, it is evident that it is likely to be penetrated deeply by the light to which it is exposed, particularly by the stronger or more intense portions thereof. The resultant printing surface after treatment will have a relatively too thick printing surface in those portions which have been thus deeply penetrated. It is very difficult, for example, to get the darker portions of a negative recorded properly without having the lighter portions of a negative registered too heavy and deep. 115

In order to overcome these disadvantages, I have discovered that excellent results may be obtained by using an emulsion colored with a color which is complementary to the exposure light. When applied to photographic printing from a negative, for example, the color will be complementary to the printing light, which generally is obtained from an incandescent electric lamp giving out blue rays. Naphthol yellow or its color equivalents in an aqueous solution 130

of substantially ten (10) grams of naphthol yellow to an ounce of liquid will give satisfactory results with such a light, as well as many other of the orange and yellow dyes.

5 If an ordinary sensitized emulsion of any desired thickness and colored as described above is exposed to such a printing light modified by any desired lights and shades as, for instance, those of a negative which it is desired to reproduce, the printing light which comes through the high lights of the negative will be absorbed or slowed down to such an extent that the printing light which comes through the dark shades of the 10 negative will be recorded in the sensitized emulsion, without a too deep penetration of the printing light coming through said high lights of the negative. If the sensitized emulsion is exposed through its transparent 15 carrier, the entire printing surface obtained after treatment will lie adjacent the carrier, which is desirable to prevent a too great thickness of printing surface corresponding to the high lights of the negative, the effect 20 of which excessive thickness is to cause the lights and shades to be too contrasting.

Many modifications of my invention will be apparent to those skilled in the art without departing therefrom or from the scope 25 of the claims, my invention not being limited to any particular emulsion or to any particular light but comprising the use of an emulsion complementary in color to the exposure light.

30 By the term "metol" in this case is meant monomethylparamidophenol sulphate or its equivalents.

What I claim is:

1. The process of forming a photographic 35 record of lights and shades capable of use as a transfer printing plate, which comprises coloring a sensitized emulsion with a color complementary to the exposure light, exposing said emulsion to the lights and shades desired to be recorded, and hardening 40 portions of emulsion adjacent the light affected sensitive content of a photographic emulsion with an agent adapted to harden said emulsion by reaction with the light affected 45 sensitive content of the emulsion, and with a neutralizing agent for said hardening agent, the relative proportions of said hardening and neutralizing agents being

such as to control selectively the effective area of influence of the hardening agent but to an extent less than the complete neutralization of said hardening agent.

2. The process specified in claim 1 in which the exposed sensitive emulsion is undeveloped prior to said treatment.

3. The process specified in claim 1 in which the hardened portions correspond to the variations of the lights and shades to which the sensitive emulsion has been exposed.

4. The process specified in claim 1 in which the sensitive content is a silver salt.

5. The process specified in claim 1 in which the hardening agent also is a developing agent.

6. The process specified in claim 1 in which the hardening agent is pyrogallic acid.

7. The process specified in claim 1 in which the neutralizing agent also is a preservative.

8. The process specified in claim 1 in which the neutralizing agent is sodium sulphite.

9. The process specified in claim 1 in which the hardening agent also is a developing agent and in which the neutralizing agent also is a preservative.

10. The process specified in claim 1 in which the hardening agent is pyrogallic acid and the neutralizing agent is sodium sulphite.

11. The process specified in claim 1 in which the sensitive content is developed at the same time the portions of emulsion adjacent the light affected sensitive emulsion are hardened.

12. The process specified in claim 1 in which said treatment is applied to a photographic emulsion mounted on and exposed through a transparent carrier.

13. The process of claim 1 in which the color is naphthol yellow.

14. The process of claim 1 in which the color is obtained from substantially ten grains of naphthol yellow to an ounce of liquid.

In testimony that I claim the foregoing, I have hereunto set my hand this 21<sup>st</sup> day of October, 1919.

ROBERT JOHN.